



3

mula as being suitable in the practice of this invention include but are not limited to the following:

TABLE I



4



The invention is best illustrated by the following examples. These examples are given by way of illustration and are not intended in any way to restrict the scope of the invention nor the manner in which it may be practiced.

### EXAMPLE I

Low carbon steel panels 0.75" x 6" are placed in a large test tube containing 8% v./v. of concentrated  $H_2SO_4$  and a equal volume of concentrated hydrochloric acid and 0.2% of the inhibitor. "Controls" are also used in which the corrosive medium contains no inhibitor. The immersion time is 6 hours and the temperature is 32° C. Methyl butynol, a commonly used acetylenic inhibitor is used for comparison. The panels are weighed before and after the corrosion period and the inhibition efficiency calculated as previously described. Table 2 gives the results.

TABLE II

|    | Compd. No. | Inhibitor                                                   | Efficiency percent |
|----|------------|-------------------------------------------------------------|--------------------|
| 40 | 1          | Methyl butynol (2-methyl-3-butyn-2-ol)                      | 94.6               |
|    | 2          | 2,2-diethyl-penta-3,4-diene-1-al                            | 97.2               |
|    | 3          | 1,2-butadiene-4-ol                                          | 96.2               |
|    | 4          | 1,2-butadiene-4-ol ethylene oxide adduct                    | 95.0               |
|    | 5          | 1-allyl-1-formyl-cyclohex-3-ene                             | 99.1               |
| 45 | 6          | 2,2-dimethyl-penta-3,4-dien-1-al                            | 94.3               |
|    | 7          | 2-methyl-2,3-butadienyltrimethylammonium chloride           | 85.3               |
|    | 8          | 1-(p-dimethylaminophenyl)-2,2-dimethyl-penta-3,4-dienol HCl | 96.5               |
|    | 9          | 1-allyl-1-carbinol-cyclohex-3-ene                           | 94.5               |
|    | 10         | 2,2-dimethylpenta-3,4-dienol                                | 88.7               |
| 50 | 11         | 2,2,5-trimethylhexa-3,4-dienal                              | 74.7               |
|    | 12         | 2,3-butadienoic acid                                        | 92.0               |

### EXAMPLE II

55 In this example the effect of concentration of the inhibitor is demonstrated. The conditions were similar to those of Example I except that 20% hydrochloric acid was used at room temperature and the corrosion period was 3.5 hours. The following table shows that very low concentrations may be used.

TABLE III

| Panel | Inhibitor,<br>percent<br>v./v. | Inhibitor                      | Efficiency,<br>percent |     |
|-------|--------------------------------|--------------------------------|------------------------|-----|
|       |                                |                                | 1-A                    | 2-A |
| 65    | 0.05                           | Methyl butynol                 | 90.1                   |     |
|       | 0.10                           | do                             | 94.2                   |     |
|       | 0.05                           | 1-allyl-1-formylcyclohex-3-ene | 98.3                   |     |
|       | 0.10                           | do                             | 98.5                   |     |

### EXAMPLE III

70 Here is shown the effect of methyl pentynol and three  
 71 allenic inhibitors on the corrosion of 0.032" thick A.C.S.  
 72 reagent grade zinc in 5% v/v. sulfuric acid. The time  
 73 was 2 hours, inhibitor concentration 0.2%, and per-  
 74 formed at room temperature. The allene inhibitor num-  
 75 bers in Table IV as well as in those examples which

follow refer to the numbers in Table II. It will be noticed that the addition of the wetting agent in the case of panel 5C slightly increased the efficiency of inhibitor No. 2.

TABLE IV

| Panel | Inhibitor                                                                           | Efficiency, percent |
|-------|-------------------------------------------------------------------------------------|---------------------|
| 1-C   | Methyl pentynol                                                                     | 84.2                |
| 2-C   | Allene #2 (2,2-diethylpenta-3,4-diene-1-al)                                         | 95.8                |
| 3-C   | Allene #5 (1-allyl-1-formylcyclo-3-ene)                                             | 95.4                |
| 4-C   | Allene #11 (2,2,5-trimethylhexa-3,4-dienal)                                         | 94.5                |
| 5-C   | Allene #2 (see above panel 2-C plus 0.1% v./v. "Surfynol" (a surface active agent)) | 96.5                |

## EXAMPLE IV

In this example aluminum (6061 alloy) strips were immersed in a solution containing 50 g./l. sodium chloride and 2% v./v. concentrated hydrochloric acid at room temperature. The time of immersion was 4 hours and the inhibitor concentration for all compounds in Table V was 0.2%. In this case the acetylenic compound appears to be more effective than the allenic compounds. When the concentration of Allene No. 11 was increased to 0.4%, the inhibition efficiency was 97.0%.

TABLE V

| Panel | Inhibitor                                   | Efficiency, percent |
|-------|---------------------------------------------|---------------------|
| 1-B   | Methylpentynol (3-methyl-1-pentyl-3-ol)     | 78.0                |
| 2-B   | Allene #2 (2,2-diethyl-penta-3,4-dien-1-al) | 66.8                |
| 3-B   | Allene #11 (2,2,5-trimethylhexa-3,4-dienal) | 57.3                |

## EXAMPLE V

Aluminum (alloy 6061) is immersed in 5% sodium hydroxide at room temperature for 65 minutes. Allene No. 5 was used at 0.1%. The efficiency was only 12% indicating that the allenic compounds do not have much promise as inhibitors for aluminum in alkaline solutions.

## EXAMPLE VI

Two steel strips are immersed in separate solutions containing 4% by volume sulfuric acid plus 0.2% by volume hydrochloric acid. One of the solutions contains 0.1% by weight of Allene No. 7. The inhibitor efficiency after 2 hours immersion is 98.2%.

## EXAMPLE VII

Steel strips were immersed in 3M  $H_2SO_4$  at room temperature for 4 hours. The efficiency of the inhibitor without and with the addition of  $7 \times 10^{-2}$  M KI is shown in Table VI.

TABLE VI

| Inhibitor and concentration: | Percent efficiency |
|------------------------------|--------------------|
| No. 11 at 0.05%              | 58.5               |
| No. 11 at 0.05%, plus KI     | 99.820             |
| No. 5 at 0.01%               | 80.6               |
| No. 5 at 0.01%, plus KI      | 99.846             |

## EXAMPLE VIII

Here is compared the effect of an allene with a compound containing a single double bond and also with a compound containing two nonadjacent double bonds. Steel panels were immersed in 20% hydrochloric acid for 22 hours at room temperature. The inhibitor concentration was 0.1% and the efficiencies are shown in Table VII.

TABLE VII

| Panel: | Inhibitor                               | Efficiency, percent |
|--------|-----------------------------------------|---------------------|
| 1-D    | Allene #5                               | 98.5                |
| 2-D    | Methyl butenol (3-methyl-1-butene-3-ol) | 58.7                |
| 3-D    | 2,5-dimethyl-1,5-hexadiene-3-ol         | 58.4                |

## EXAMPLE IX

The following test was performed as an indicative example of vapor inhibition. Several layers of filter paper

were laid on the bottom of three 1 liter tall form beakers. In all cases the filter paper was saturated with water. About 0.5 g. of Allene No. 2 was added to the wet filter paper in one beaker and 0.5 g. of Allene No. 3 (see Example I) to that in another beaker. No inhibitor was added to the third beaker. Clean steel panels were then placed upright in the three beakers and these placed in a laboratory where the atmosphere was acidic and humid for four weeks. Once a week the filter papers were rewetted with water or water plus inhibitor. At the end of four weeks the steel in the beaker containing no inhibitor had become tarnished with yellow rust while the panels in the beakers containing the inhibitors were relatively tarnish-free.

From the previous examples, it is obvious that the effectiveness of allenic compounds as inhibitors can be equal or greater than that of acetylenic compounds. In this respect they resemble the acetylenic compound more than they do simple olefins or conjugated diolefins. It also appears that those allenes with a terminal double bond are more effective as inhibitors for steel than those which do not have the terminal double bond. In general this is also true for olefins and acetylenic compounds.

Due to the volatility of some of the allenic alcohols and aldehydes at elevated temperatures, it is generally advisable that the inhibitor containing solution be held at a temperature of less than 130° F. This restriction of course is not necessary for the allenic amines which form nonvolatile salts.

Allenic compounds used in the practice of this invention can be prepared by various methods taught in the prior art, including British Pat. 971,751; Bailey & Pfeifer, J. Org. Chem., 20, 1337-41 (1955); Eglinton et al., J. Chem. So., 3197-3200 (1954). Typical procedures are given below for various typical compounds.

## 1-allyl-2,2-demethyl-3,4-pentadienal

A solution containing 0.15 mole of allylmagnesium bromide in 250 ml. of ether is added dropwise with cooling to a solution of 16.5 g. (0.15 mole) of 2,2-dimethyl-3,4-pentadienal in 30 ml. of ether. After the reaction is complete the mixture is shaken with dilute hydrochloric acid. The ether phase is separated, washed with fresh water and dried over sodium sulfate. Upon evaporation of the ether and distillation of the residue, 8.0 g. of product is collected which boils at 80-1° C. at 10 mm. Hg. Infrared analysis shows strong adsorption at 5.1 microns, which is characteristic of the allenic group, and strong absorptions for hydroxyl and allyl groups.

## 1-(p-dimethylaminophenyl)-2,2-dimethyl-3,4-pentadienol

An ethereal solution containing 0.1 mole of p-dimethylaminophenyl lithium is added over a 0.5 hour period, at ice bath temperature, to an ethereal solution of 11.0 g. (0.1 mole) of 2,2-dimethyl-3,4-pentadienol. After the reaction is complete the mixture is cautiously hydrolyzed with an excess of water. The ether phase is separated and extracted with dilute hydrochloric acid. The combined extracts are washed with fresh ether and then neutralized with dilute sodium hydroxide. The product is extracted several times with ether and the combined extracts are dried over sodium sulfate. The product is precipitated from ether solution as the hydrochloric salt with anhydrous hydrogen chloride. A white solid, 15.0 g., is collected. Infrared analysis shows strong allenic absorption at 5.1 microns, and strong absorptions for hydroxyl, amino and phenyl groups.

## 1-formyl-1-allylencyclohexene-3

A mixture of 23.0 g. (0.41 mole) of propargyl alcohol, 45.3 g. (0.41 mole) of 1-formylcyclohexene-3, 0.1 g. of hydroquinone and 0.1 g. of p-toluene sulfonic acid in 60 ml. of benzene is heated at reflux for 5 hours. The water of reaction is collected in a Dean-Stark trap. Fractionation of the mixture affords 22.0 g. of product boiling at

71° C. at 3 mm. Hg. Infrared analysis shows strong absorption for the allenyl, aldehyde and cyclohexene groups.

1-hydroxymethyl-1-allenylcyclohexene-3

To a solution of 10.3 g. (0.07 mole) of 1-formyl-1-allenylcyclohexene-3 and 7.0 ml. of 40% formaldehyde solution in 25 ml. of methanol is added 8.4 g. of 50% sodium hydroxide solution over 15 minutes at 35-50° C. The mixture is then heated at 60° C. for 3 hours and poured into 300 ml. of water. The mixture is extracted with three 50 ml. portions of benzene. The combined extracts are dried over sodium sulfate and distilled. By this procedure, 6.5 g. of product, boiling at 95-6° C. at 3 mm. Hg is collected. The infrared analysis shows strong absorptions for the allenic, hydroxyl and cyclohexenyl groups.

3,6-dioxa-8,9-decadien-1-ol

A mixture of 1.0 g. of powdered potassium hydroxide and 40 ml. of isopropanol is stirred at reflux until the solids are dissolved. The solution is cooled at 25° C. and 10.0 g. (0.143 mole) of 2,3-butadiene-1-ol is added. With agitation, 13.2 g. (0.3 mole) of ethylene oxide is passed into the solution over a 30 minute period. The reaction temperature is maintained at 25-35° C. by intermittent cooling. After the addition is complete the mixture is stirred at 40-50° C. for 1 hour and then at 30° C. for an additional 2 hours. The catalyst is neutralized with hydrochloric acid and the mixture is filtered through a bed of Filter Cel. The isopropanol and unreacted 2,3-butadiene-1-ol are distilled from the mixture to a maximum pot temperature of 80° C. at 10 mm. Hg. A dark orange, water soluble oil, 19.5 g., is obtained. Infrared analysis indicates strong absorption for the allenic, ether, and hydroxyl groups.

I claim:

1. A corrosion inhibited aqueous acid solution containing an effective corrosion inhibiting amount of an allenic compound of the formula



wherein

R', R<sup>2</sup> and R<sup>3</sup> are selected from the group consisting of hydrogen and methyl,

X is selected from the group consisting of —CHO; —COOH; —CH<sub>2</sub>OH; —C(R<sup>4</sup>)<sub>2</sub>CHO;



R<sup>4</sup> is selected from the group consisting of hydrogen or an alkyl radical of 1-4 carbon atoms, or two such R<sup>4</sup>'s can be aliphatic hydrocarbon divalent radicals joined to form a six-membered cycloaliphatic ring with the carbon of the formula,

R<sup>5</sup> is selected from the group consisting of hydrogen and an alkyl radical of 1-4 carbon atoms,

R<sup>6</sup> is a divalent saturated aliphatic hydrocarbon radical of 2-6 carbon atoms,

Ar is selected from the group consisting of phenylene, naphthylene, diphenylene or an alkylene having 1-4 carbon atoms, and

n is an integer of from 1-10.

2. A corrosion inhibited aqueous acid solution as stated in claim 1 wherein said allenic compound is present in a concentration of between about 0.005 and 4 grams per liter of solution.

3. A corrosion inhibited aqueous acid solution containing an effective corrosion inhibiting amount of 2,2-diethyl-penta-3,4-diene-1-al.

4. A corrosion inhibited aqueous acid solution contain-

75

ing an effective corrosion inhibiting amount of 1-allenyl-1-formyl-cyclohex-3-ene.

5. A corrosion inhibited aqueous acid solution containing an effective corrosion inhibiting amount of 2,3-butadienoic acid.

6. A method of inhibiting corrosion of ferrous, zinc or aluminum containing materials in acidic aqueous solutions which comprises dissolving in said aqueous solutions between about 0.005 and 4 grams of an allenic compound per liter of solution, said allenic compound being of the formula



wherein

R', R<sup>2</sup> and R<sup>3</sup> are selected from the group consisting of hydrogen and methyl,

X is selected from the group consisting of —CHO; —COOH; —CH<sub>2</sub>OH; —C(R<sup>4</sup>)<sub>2</sub>CHO;



R<sup>4</sup> is selected from the group consisting of hydrogen or an alkyl radical of 1-4 carbon atoms, or two such R<sup>4</sup>'s can be aliphatic hydrocarbon divalent radicals joined to form a six-membered cycloaliphatic ring with the carbon of the formula

R<sup>5</sup> is selected from the group consisting of hydrogen and an alkyl radical of 1-4 carbon atoms,

R<sup>6</sup> is a divalent saturated aliphatic hydrocarbon radical of 2-6 carbon atoms,

Ar is selected from the group consisting of phenylene, naphthylene, diphenylene or an alkylene having 1-4 carbon atoms, and

n is an integer from 1-10.

7. A method of inhibiting corrosion of ferrous, zinc or aluminum containing materials in acidic aqueous solutions which comprises dissolving in said aqueous solutions between about 0.005 and 4 grams per liter of 2,2-diethyl-3,4-diene-1-al.

8. A method of inhibiting corrosion of ferrous, zinc or aluminum containing materials in acidic aqueous solutions which comprises dissolving in said aqueous solutions between about 0.005 and 4 grams per liter of 1-allenyl-1-formyl-cyclohex-3-ene.

9. A method of inhibiting corrosion of ferrous, zinc or aluminum containing materials in acidic aqueous solutions which comprises dissolving in said aqueous solutions between about 0.005 and 4 grams per liter of 2,3-butadienoic acid.

10. A method of inhibiting corrosion or tarnishing of ferrous, zinc or aluminum containing materials in a corrosive atmosphere contacting said metal containing materials with a corrosion inhibiting amount of an allenic compound in a vapor phase, said allenic compound being of the formula



wherein

R', R<sup>2</sup> and R<sup>3</sup> are selected from the group consisting of hydrogen and methyl,

X is selected from the group consisting of —CHO; —COOH; —CH<sub>2</sub>OH; —C(R<sup>4</sup>)<sub>2</sub>CHO;



**9**—C(R<sup>4</sup>)<sub>2</sub>N(R<sup>5</sup>)<sub>3</sub>Cl; —C(R<sup>4</sup>)<sub>2</sub>(OR<sup>6</sup>)<sub>n</sub>OH; —C<sub>5</sub>H<sub>4</sub>N;and —C<sub>5</sub>H<sub>10</sub>N,

R<sup>4</sup> is selected from the group consisting of hydrogen or an alkyl radical of 1-4 carbon atoms, or two such R<sup>4</sup>'s can be aliphatic hydrocarbon divalent radicals joined to form a six-membered cycloaliphatic ring with the carbon of the formula,

R<sup>5</sup> is selected from the group consisting of hydrogen or an alkyl radical of 1-4 carbon atoms,

R<sup>6</sup> is a divalent saturated aliphatic hydrocarbon radical of 2-6 carbon atoms,

Ar is selected from the group consisting of phenylene,

**10**

naphthylene, diphenylene or an alkylene having 1-4 carbon atoms, and

*n* is an integer from 1-10.

**References Cited****UNITED STATES PATENTS**

3,148,223 9/1964 Jacobs et al. ----- 260—653.5

RICHARD D. LOVERING, Primary Examiner

I. GLUCK, Assistant Examiner

U.S. Cl. X.R.

252—148, 396